

# United States Patent Office

2,796,355

Patented June 18, 1957

1

2,796,355

## NON-FOAMING WAX

Francis J. Higgins, Ponca City, Okla., assignor to Continental Oil Company, Ponca City, Okla., a corporation of Delaware

No Drawing. Application August 9, 1954,

Serial No. 448,780

8 Claims. (Cl. 106—270)

This invention relates to compositions for controlling foaming of waxes and more particularly for inhibiting foaming of waxes used in coating operations.

As is well known to those familiar with the art of coating paper with wax, one method in common practice is to dip the paper in a hot molten wax bath whereby the paper is coated with the wax and rendered waterproof. It is also known that in general molten waxes have marked foaming tendencies and as a result foaming problems must be dealt with. When this foam is stable it solidifies on the surface of the paper with the result that the paper is only partially covered with wax. If a container prepared from such paper is filled with a liquid, the liquid penetrates the paper through the areas which had been covered by the foam thereby weakening the paper container causing bulging and leakers. Furthermore, such a container is unattractive.

It is, therefore, a principal object of the present invention to provide a non-foaming wax. Another object of my invention is to provide a combination of certain esters with an alkali metal fatty acid soap in critical ratios which combination eliminates foaming tendencies of waxes. A further object of the present invention is to provide a non-foaming wax containing a minor amount of this critical combination of additives. Other objects and advantages of the present invention will become apparent as the invention is hereinafter more thoroughly described.

I have found that the foaming tendencies of wax can be sharply reduced economically and simply. This can be accomplished by adding to the wax a minor amount of certain esters and certain fatty acid soaps within a critical range of ratios by weight as an antifoamant. The present invention resides primarily in an antifoamant composition consisting of a major proportion of an ester of a polyhydric alcohol used in combination with a minor proportion of a fatty acid soap which composition is then incorporated in a wax. Suitable esters are those prepared by reacting a fatty acid such as lauric, myristic, palmitic, stearic, oleic, ricinoleic, and the like, with a polyhydric alcohol such as ethylene glycol, propylene glycol, diethylene glycol, glycerine, polyglycols, mannitol, sorbitol, and the like. Typical esters are glycerol monostearate, diglycol monostearate, polyglycol palmitate. Of the many suitable esters available, monoglycerides are preferred. Suitable soaps include potassium and lithium fatty acid soaps. Of these two types of soaps, potassium fatty acid soaps are preferred because they are more effective, cheaper, and available in greater quantities than the corresponding lithium soaps.

As used herein and in the appended claims the term wax includes paraffin wax as that term is commonly understood and in addition the paraffin wax may contain such materials as higher boiling distillate waxes, microcrystalline wax, polyethylenes, and perhaps other additives. In general, the term "paraffin wax" is used to define the hard, crystalline wax commonly obtained from petroleum distillates, derived from mineral oils of the mixed base or paraffin base type. By the present refining methods, crude petroleum oil is subjected to distillation whereby it is separated into a series of fractions known as "paraffin distillates." The wax is separated from the paraffin distillate by chilling and filtering or

2

by the use of a solvent, as for example, propane or a ketone such as methyl ethyl ketone. The wax obtained by either of these two methods contains from 10 to 50 percent oil and is generally referred to as "slack wax."

5 This slack wax is subjected to a "sweating operation" to remove the oil. The resulting wax usually contains 3 to 6 percent oil, but by proper sweating the oil content may be reduced to less than 1 percent. Also, the oil content may be reduced to an acceptable value by other methods such as solvent de-oiling or press de-oiling. The final product is known as "refined wax" or "paraffin wax" and is graded according the tensile strength, melting point, oil content, hardness, etc.

10 The quantity of the antifoamant composition added to the wax will depend upon a number of factors. Thus, the exact quantity of the antifoamant added will depend upon the particular ester and fatty acid soap and the relative quantities of each making up the antifoamant. In general, the antifoamant may be employed to advantage in wax 15 in amounts ranging from about 0.03 to about 0.3 percent by weight, of the wax composition. Quantities less than 0.03 percent are insufficient to reduce the foaming characteristics of the wax and if the amount is in excess of 0.3 percent the result is unsatisfactory. A preferred range is from about 0.1 to about 0.2 percent by weight of the wax composition. Suitable quantities of the fatty acid soap in comparison to the amount of ester ranges from about 3 to 10 percent of the former with the remainder of the antifoamant being made up of the ester. 20 I prefer, however, to use about 5 to 7 percent of the soap and from 95 to 93 percent of the ester as the antifoamant composition.

25 While I do not wish to be bound by any theory as to how my results are produced, I believe that the correct explanation of these results is substantially as follows: The ester acts as a coupling agent and hereinafter will be identified as a coupling agent which affects the mutual limited solubility between the soap and wax that is required to inhibit foam formation.

30 The relative effectiveness of the various soap-coupling agent combinations of my invention in preventing foam formation in a wax may be demonstrated by means of the following foam tests. Briefly, the foam test consists of introducing a stream of air at a fixed rate into a measured quantity of wax at 175° F. by means of a fritted glass gas dispersion tube. After a predetermined time the volume of foam produced is measured as well as the time required for the bulk of the foam to dissipate after the air flow is stopped. This method is a modification of 35 A. S. T. M. method D 892-46T. The base waxes A, B, C, and D used in the examples are basically of the same composition, the melting points of which are 126.6, 125, 125.5 and 126.9° F. respectively as determined by the A. S. T. M. melting point method. They differ only in 40 their foaming tendencies.

45 In the following specific examples, there are illustrated by means of this foaming test the advantageous results obtained by incorporating in a wax the antifoamants of my invention.

## EXAMPLE 1

|                                                    | Foam        |              |
|----------------------------------------------------|-------------|--------------|
|                                                    | Vol. in ml. | Time in Sec. |
| 65                                                 |             |              |
| Wax B (control)                                    | 24.0        | 8.7          |
| 100 parts Wax B, 0.1 part antifoamant <sup>1</sup> | 1.0         | 1.0          |
| Wax C (control)                                    | 32.0        | 14.0         |
| 100 parts Wax C, 0.1 part antifoamant <sup>1</sup> | 9.0         | 4.9          |

<sup>1</sup> Mixture of 5 parts of potassium laurate with 95 parts of glyceryl monolaurate.

Several other waxes have been tested in a similar manner, both alone and with the antifoamant and have shown the same foam reduction as indicated in the foregoing example. In addition to this laboratory data, several commercial machine coating experiments have been conducted and a very decided reduction or elimination of foam on the coated paper was observed.

Example 2 demonstrates that the components of the anti-foamant, potassium laurate and glyceryl monolaurate, do not have foam suppressing properties when used alone.

5

[Antifoamant composition: 10% potassium laurate; 90% glyceryl monolaurate.]

|                                        | Foam        |              |
|----------------------------------------|-------------|--------------|
|                                        | Vol. in ml. | Time in Sec. |
| Wax B (control)                        | 24.0        | 8.7          |
| 100 parts Wax B, 0.01 part antifoamant | 23.5        | 9.2          |
| 100 parts Wax B, 0.05 part antifoamant | 22.5        | 7.4          |
| 100 parts Wax B, 0.1 part antifoamant  | 9.0         | 4.7          |

[Antifoamant composition: 3% potassium laurate; 97% glyceryl monolaurate.]

### EXAMPLE 2

|                                                           | Foam        |              |
|-----------------------------------------------------------|-------------|--------------|
|                                                           | Vol. in ml. | Time in Sec. |
| Wax D (control)                                           | 23.5        | 8.0          |
| 100 parts Wax D, 0.01 part potassium laurate <sup>1</sup> | 26.0        | 11.4         |
| 100 parts Wax D+0.1 part glyceryl monolaurate             | 23.0        | 9.4          |

<sup>1</sup> Difficultly soluble in wax.

The range of effective foam suppression of a mixture of 6-7 percent potassium laurate with 94-93 percent glyceryl monolaurate is illustrated by the data in Table I.

Table I

|                                        | Foam        |              |
|----------------------------------------|-------------|--------------|
|                                        | Vol. in ml. | Time in Sec. |
| Wax B (control)                        | 24.0        | 8.7          |
| 100 parts Wax B, 0.02 part antifoamant | 22.0        | 10.3         |
| 100 parts Wax B, 0.03 part antifoamant | 21.0        | 10.2         |
| 100 parts Wax B, 0.04 part antifoamant | 3.5         | 3.7          |
| 100 parts Wax B, 0.05 part antifoamant | 1.0         | 1.0          |
| Wax A (control)                        | 21.5        | 10.3         |
| 100 parts Wax A, 0.1 part antifoamant  | 2.0         | 1.0          |
| 100 parts Wax A, 0.2 part antifoamant  | 2.0         | 1.0          |
| 100 parts Wax A, 0.3 part antifoamant  | 4.0         | 12.8         |

In order to demonstrate that a proper combination of soap and coupling agent is required to inhibit foam effectively in a wax, the following data are presented.

[Antifoamant composition: 20% potassium laurate; 80% glyceryl monolaurate.]

|                                        | Foam        |              |
|----------------------------------------|-------------|--------------|
|                                        | Vol. in ml. | Time in Sec. |
| Wax B (control)                        | 24.0        | 8.7          |
| 100 parts Wax B, 0.01 part antifoamant | 25.0        | 9.0          |
| 100 parts Wax B, 0.05 part antifoamant | 25.0        | 10.0         |
| 100 parts Wax B, 0.1 part antifoamant  | 21.0        | 7.8          |

[Antifoamant composition: 15% potassium laurate; 85% glyceryl monolaurate.]

|                                        | Foam        |              |
|----------------------------------------|-------------|--------------|
|                                        | Vol. in ml. | Time in Sec. |
| Wax B (control)                        | 24.0        | 8.7          |
| 100 parts Wax B, 0.01 part antifoamant | 25.0        | 10.4         |
| 100 parts Wax B, 0.05 part antifoamant | 27.0        | 12.4         |
| 100 parts Wax B, 0.1 part antifoamant  | 26.0        | 10.2         |

10

15

20

25

30

35

40

45

55

60

65

[Antifoamant composition: 10% potassium laurate; 90% glyceryl monolaurate.]

|                                        | Foam        |              |
|----------------------------------------|-------------|--------------|
|                                        | Vol. in ml. | Time in Sec. |
| Wax B (control)                        | 24.0        | 8.7          |
| 100 parts Wax B, 0.01 part antifoamant | 23.5        | 9.2          |
| 100 parts Wax B, 0.05 part antifoamant | 22.5        | 7.4          |
| 100 parts Wax B, 0.1 part antifoamant  | 9.0         | 4.7          |

[Antifoamant composition: 3% potassium laurate; 97% glyceryl monolaurate.]

|                                        | Foam        |              |
|----------------------------------------|-------------|--------------|
|                                        | Vol. in ml. | Time in Sec. |
| Wax B (control)                        | 24.0        | 8.7          |
| 100 parts Wax B, 0.05 part antifoamant | 25.5        | 12.7         |
| 100 parts Wax B, 0.1 part antifoamant  | 3.0         | 3.3          |
| 100 parts Wax B, 0.2 part antifoamant  | 1.5         | 2.6          |

[Antifoamant composition: 2% potassium laurate; 98% glyceryl monolaurate.]

|                                       | Foam        |              |
|---------------------------------------|-------------|--------------|
|                                       | Vol. in ml. | Time in Sec. |
| Wax B (control)                       | 24.0        | 8.7          |
| 100 parts Wax B, 0.1 part antifoamant | 22.5        | 11.2         |
| 100 parts Wax B, 0.2 part antifoamant | 25.5        | 13.8         |
| 100 parts Wax B, 0.3 part antifoamant | 25.0        | 12.1         |

[Antifoamant composition: 1% potassium laurate; 99% glyceryl monolaurate.]

|                                       | Foam        |              |
|---------------------------------------|-------------|--------------|
|                                       | Vol. in ml. | Time in Sec. |
| Wax B (control)                       | 24.0        | 8.7          |
| 100 parts Wax B, 0.1 part antifoamant | 26.5        | 11.8         |
| 100 parts Wax B, 0.2 part antifoamant | 25.5        | 14.1         |
| 100 parts Wax B, 0.3 part antifoamant | 24.5        | 9.3          |
| 100 parts Wax B, 0.4 part antifoamant | 26.5        | 14.3         |

As is apparent from the data of Example 3 below my antifoamant compositions are effective in inhibiting the foaming of wax mixtures. This is highly desirable because as is well known that in a blend of two or more waxes the foaming tendencies of the resulting blend increases as the amount of higher melting point wax in the blend increases.

### EXAMPLE 3

|                                                                                       | Foam        |              |
|---------------------------------------------------------------------------------------|-------------|--------------|
|                                                                                       | Vol. in ml. | Time in Sec. |
| Wax E (M. P. 123.6° F.)                                                               | 4.5         | 1.3          |
| Wax E (100 parts)+a microcrystalline wax, M. P. 175° F. (3 parts)                     | 15.0        | 7.1          |
| 100 parts mixture Wax E and microcrystalline wax+0.1 part of antifoamant <sup>1</sup> | 2.5         | 1.0          |

<sup>1</sup> 5 parts potassium laurate and 95 parts glyceryl monolaurate.

Table II illustrates that other esters may be used in this invention. It also includes data showing that lithium soap is effective but that soaps composed of fatty acids of sodium, calcium, and aluminum have no foam suppressing properties when used in combination with various esters. The data of Table II were obtained by adding 0.1 part of the antifoamant to 100 parts of wax wherein the antifoamant consisted of 5% soap and 95% of the coupling agent.

**5**  
**Table II**  
**EFFICIENCY OF DIFFERENT SOAP-CO尤LING AGENT COMBINATIONS AS AN ANTIFOAMANT**

| Wax | Antifoamant Composition         |                              | Foam         |               | 5  |
|-----|---------------------------------|------------------------------|--------------|---------------|----|
|     | Soap                            | Coupling Agent               | Vol.,<br>ml. | Time,<br>Sec. |    |
| C   | None                            | None                         | 32.0         | 14.0          |    |
| C   | Lithium laurate                 | Glyceryl monolaurate         | 20.0         | 6.6           |    |
| C   | Potassium myristate             | do                           | 1.5          | 1.5           |    |
| D   | None                            | Glyceryl monostearate        | 23.5         | 8.0           |    |
| D   | Potassium myristate             | Glyceryl mono-oleate         | 8.5          | 3.2           |    |
| D   | do                              | Glyceryl monolaurate         | 31.0         | 12.4          |    |
| O   | None                            | None                         | 32.0         | 14.0          |    |
| C   | Potassium laurate               | Glyceryl monolaurate         | 9.0          | 4.9           |    |
| D   | None                            | None                         | 23.5         | 8.0           | 15 |
| D   | Potassium laurate               | Glyceryl monolaurate         | 1.0          | 1.0           |    |
| D   | do                              | Glyceryl monostearate        | 1.0          | 1.0           |    |
| D   | do                              | Glyceryl mono-oleate         | 4.0          | 3.6           |    |
| O   | None                            | None                         | 32.0         | 14.0          |    |
| C   | Potassium laurate               | Hydrogenated Castor oil      | 26.5         | 8.3           |    |
| O   | do                              | Hydrogenated lard            | 25.0         | 7.4           |    |
| C   | do                              | Hydrogenated fish oil        | 27.0         | 8.4           |    |
| O   | do                              | Hydrogenated tallow          | 23.0         | 7.2           |    |
| D   | None                            | None                         | 23.5         | 8.0           |    |
| D   | Potassium laurate               | Polyethylene glycol stearate | 14.0         | 5.4           |    |
| D   | do                              | Ethylene glycol stearate     | 16.0         | 6.7           |    |
| D   | None                            | None                         | 23.5         | 8.0           | 25 |
| D   | Potassium palmitate             | Glyceryl monolaurate         | 2.0          | 1.0           |    |
| D   | do                              | Glyceryl monostearate        | 15.0         | 3.5           |    |
| D   | do                              | Glyceryl mono-oleate         | 15.0         | 6.4           |    |
| D   | None                            | None                         | 23.5         | 8.0           |    |
| D   | Potassium stearate              | Glyceryl monolaurate         | 24.0         | 8.1           |    |
| D   | do                              | Glyceryl monostearate        | 23.0         | 6.8           | 30 |
| D   | do                              | Glyceryl mono-oleate         | 15.0         | 6.0           |    |
| O   | None                            | None                         | 32.0         | 14.0          |    |
| O   | Potassium oleate                | Glyceryl monolaurate         | 6.0          | 4.0           |    |
| O   | None                            | None                         | 32.0         | 14.0          |    |
| C   | Sodium myristate                | Glyceryl monolaurate         | 35.0         | 14.5          |    |
| D   | None                            | None                         | 23.5         | 8.0           |    |
| D   | Sodium laurate                  | Glyceryl monolaurate         | 24.0         | 8.4           |    |
| D   | do                              | Glyceryl monostearate        | 23.5         | 11.6          |    |
| O   | None                            | None                         | 32.0         | 14.0          | 35 |
| O   | Sodium laurate                  | Glyceryl monolaurate         | 36.0         | 12.3          |    |
| C   | None                            | None                         | 32.0         | 14.0          |    |
| O   | Sodium palmitate                | Glyceryl monolaurate         | 33.5         | 12.1          |    |
| O   | Sodium stearate                 | Glyceryl monostearate        | 30.5         | 10.0          |    |
| O   | do                              | do                           | 42.0         | 13.5          |    |
| O   | None                            | None                         | 32.0         | 14.0          |    |
| O   | Calcium laurate                 | Glyceryl monolaurate         | 34.0         | 19.0          | 40 |
| O   | Aluminum dilaurate              | do                           | 29.0         | 13.5          |    |
| C   | Ether washed aluminum dilaurate | do                           | 28.0         | 9.1           |    |
| D   | None                            | None                         | 23.5         | 8.0           |    |
| D   | Aluminum stearate               | Glyceryl monostearate        | 21.5         | 7.1           |    |

Methods for preparing the soaps and the esters used in this invention are well known to those skilled in the art. One such method is substantially as follows: The fatty acid is mixed with glycerine, potassium hydroxide added after which the mixture is heated until esterification is accomplished. In this process the potassium soap of the corresponding fatty acid is also produced.

Commercial mono glycerides containing di and tri-glycerides are satisfactory for use in this invention. For example, when coconut oil which is a mixture of tri-glycerides of several fatty acids is used it is desirable to add excess glycerine with a suitable catalyst such as potassium hydroxide then heat the mixture in order to

produce the self emulsifying grade of monoglycerides. Such a product will contain mixtures of monoglycerides and potassium soaps as well as some di, and triglycerides.

While particular embodiments of the invention have been described, it will be understood, of course, that the invention is not limited thereto since many modifications may be made, and it is, therefore, contemplated to cover by the appended claims any such modifications as fall within the true spirit and scope of the invention.

The invention having thus been described, what is claimed and desired to be secured by Letters Patent is:

1. A substantially anhydrous wax composition of improved antifoaming properties intended to be used in the molten state consisting essentially of a paraffin wax and from about .03 to .3 part of an antifoamant composition per 100 parts of said wax wherein said antifoamant comprises an ester formed by reacting a fatty acid containing 11 to 20 carbon atoms with a polyhydric alcohol containing 2 to 18 carbon atoms and an alkali metal fatty acid soap wherein the alkali metal is selected from the group consisting of potassium and lithium wherein the relative proportion of said ester and said alkali metal fatty acid soap in said antifoamant composition varies from 90 to 97 percent and 10 to 3 percent respectively.

2. A substantially anhydrous wax composition of improved antifoaming properties intended to be used in the molten state consisting of .1 to .2 part of an antifoamant composition per 100 parts of a paraffin wax wherein said antifoamant comprises an ester formed by reacting a fatty acid containing 11 to 20 carbon atoms with a polyhydric alcohol containing 2 to 18 carbon atoms and an alkali metal fatty acid soap wherein the alkali metal is selected from the group consisting of potassium and lithium wherein the relative proportion of said ester and said alkali metal fatty acid soap in said antifoamant composition vary from 93 to 95 percent and 7 to 5 percent respectively.

3. The product of claim 1 wherein the ester is a monoglycerine.

4. The product of claim 1 wherein the ester is glyceryl monolaurate.

5. The product of claim 1 wherein the alkali metal fatty acid soap is potassium laurate.

6. The product of claim 1 wherein the alkali metal fatty acid soap is potassium myristate.

7. The product of claim 1 wherein the alkali metal fatty acid soap is potassium palmitate.

8. The product of claim 1 wherein the alkali metal fatty acid soap is lithium laurate.

#### References Cited in the file of this patent

#### UNITED STATES PATENTS

- |           |                 |               |
|-----------|-----------------|---------------|
| 2,346,928 | Lightpipe       | Apr. 18, 1944 |
| 2,390,212 | Fritz           | Dec. 4, 1945  |
| 2,577,643 | Young et al.    | Dec. 4, 1951  |
| 2,658,004 | Eldridge et al. | Nov. 3, 1953  |
| 2,668,150 | Luvise          | Feb. 2, 1954  |